

## UNITED STATES PATENT OFFICE.

FRANK M. DARROW, OF JACKSON, CALIFORNIA.

## ORE-TREATING PROCESS.

No Drawing.

Application filed August 1, 1922. Serial No. 579,037.

*To all whom it may concern:*

Be it known that I, FRANK M. DARROW, a citizen of the United States, residing at Jackson, county of Amador, State of California, have invented certain new and useful Improvements in Ore-Treating Processes; and I do declare the following to be a full, clear, and exact description of the same.

This invention relates to improvements in ore-treating processes of a hydro-metallurgical nature, and particularly to a process for the treatment of certain gold and silver ores which contain elements which prevent the precious metals from being isolated and removed from the ores by the ordinary cyaniding treatments or processes.

The steps usually taken in carrying out these ordinary processes are well known and need not be set forth here. Most ores yield readily to such treatments, but occasionally an ore is found which contains one or more elements which have a tendency to either prevent the economical dissolution of the precious metals, or have a decomposing or precipitating action prematurely removing the dissolved metals from the cyanide solution. This behaviour is manifested mainly by those ores which contain graphitic-schists or other metamorphosed carbonaceous matter, which when brought in contact with the ordinary cyanide solution has the detrimental effect of prematurely precipitating out the gold and silver from the solution. Since the once precipitated metals cannot be redissolved by any strength of cyanide solution, the latter when withdrawn contains such a small percentage of the precious metals as to render cyaniding unprofitable.

I am aware that recovery of the precious contents of such ores has been attempted as for instance by drying and roasting the ores, after which cyaniding can be readily carried out, but the expense of labor and fuel incident to such treatment renders this method uneconomical and impractical from a commercial standpoint.

Other methods have also been tried out, but they all, as far as I am aware, are defective, in that they incur too much expense or fail to recover a sufficient percentage of the precious metals which it is desired to save.

The principal object of my invention

therefore is to provide an ore-treatment process for ores of the above named character by means of which the ores may first be successfully and economically treated in the wet state and left in such a condition that the ordinary cyaniding process may then be likewise successfully and economically applied thereto.

A further object is to provide such a process as may be successfully used in the treatment of "oil flotation" concentrates, containing graphitic or carbonaceous matter.

In the past, large quantities of refractory carbonaceous gold ores have been rejected into tailing-piles, but these old piles may now be handled over again and treated by my process, and an economic extraction obtained.

In general my process consists in first pulverizing the ores, and then treating them with alkaline salts of certain organic acids, after which the ores may be cyanided in the ordinary way and a good extraction of the precious metals obtained.

The best results are obtained by treating the pulverized ore or ore-pulp with a weak solution of certain of the sodium or potassium salts of organic acids, such as the higher members of the series  $C_nH_{2n}O_2$ , as myristic, lauric, stearic or palmitic acids; also the salts of oleic acid and certain others that form alkali salts.

Since these organic compounds form the main constituent of ordinary commercial laundry soaps, in practice, common soap, or by-products from soap works, or other saponaceous substances, can be used as the source of the necessary organic salts.

If desired however the saponaceous substance may be prepared especially for my purpose so as to contain the most desirable elements.

As previously stated, the carbonaceous matter in the ores to be thus treated interferes with the effectual solution of the gold and silver, and I have found by experiment that this interference can be overcome by the use of certain organic compounds, particularly those of the nature above stated.

I take advantage of this however in my process, by feeding the organic chemical to the pulp, after which the carbonaceous matter ceases to interfere, and will permit the

gold and silver in the ore to be dissolved and extracted when the usual cyaniding process is applied.

In practice, it may be found beneficial to 5 add an acid to some ores, in combination with the saponaceous matter, or before or after the latter. In other instances, it may be desirable to keep the pulp either neutral or basic. Again, with some ores this organic 10 chemical may be added and carried along with the cyanide in solution.

When it is desired to settle or filter the pulp, some agent such as lime or other coagulating agent should be used.

15 After the gold has been dissolved should the soap in solution be found to interfere with the recovery of the precious metals from the cyanide solution, it may be removed by adding calcium chloride or aluminum sulphate to render the soap insoluble, or some other substance, to decompose the soap.

If desired, the soapy compound in solution may be removed and recovered for future use with other batches of ore by washing, filtration, settling, or any other means, suitable for the purpose.

It will be noted that apart from grinding the ore, which is necessary in any event for 30 the cyaniding of the ore, no violent action or mechanical expenditure of power is necessary in carrying out my process, since the reagents that I use are very soluble in water, and when dissolved and fed in liquid form 35 to the pulp under treatment may merely diffuse themselves through the pulp and thus mingle with the elements therein to accomplish their purpose.

Unlike an oleaginous substance these soluble 40 reagents do not interfere with mercury amalgamation, should it be desirable to use this method of gold recovery along with the cyaniding process.

This kind of ore is sometimes treated by 45 the "oil-flotation" method to remove the deleterious graphitic matter in a frothy concentrate, after which the oil-flotation residue is subjected to the usual cyaniding treatment.

50 As practised however, this process is unsatisfactory inasmuch as a large percentage of the precious metal content goes into the frothy concentrates along with the deleterious matter, since the metals are mingled 55 directly with such matter. Such a concentrate could not ordinarily be then treated by the cyanide method, but my process may be applied to these concentrates with excellent results as regards the percentage of precious 60 metals recovered when the concentrates, after being treated by my process, are subject to a cyanide solution.

While this specification sets forth in detail the present and preferred steps of the 65 process, still in practice such deviations

from such detail may be resorted to as do not form a departure from the spirit of the invention as defined by the appended claims.

Having thus described my invention, what I claim as new and useful and desire 70 to secure by Letters Patent, is:—

1. The process of treating gold and silver bearing tailings containing a substance tending to join to and hold the precious metals within the pulp, consisting of neutralizing such tendency of said substance by feeding into the pulp a solution of the sodium or potassium salts of the organic acids of the higher members of the series  $C_nH_{2n}O_2$ , and extracting the precious metals 80 by cyanide solution.

2. The process of treating gold and silver ores containing a substance tending to hold the precious metals within the ore, consisting of feeding directly into the ore an aqueous solution of a soluble soap, and employing cyanide to extract the precious metals.

3. The process of treating gold and silver bearing ores containing some materials interfering with the removal of the precious metals from the ore by ordinary cyanidation, consisting of overcoming such interference by means of a saponified substance of a soluble nature, and cyaniding the ore 90 for its precious metals.

4. The process of treating gold and silver bearing ores containing a re-precipitating element, consisting of, first treating the ore in a pulverized condition with a soap solution to an amount in excess of that necessary to neutralize the re-precipitating element, then recovering or removing the excess of said soap solution, and finally subjecting the ore thus treated to a cyanide treatment.

5. The process of treating gold and silver ores containing carbonaceous matter, consisting of treating the ore in a pulverized condition with a soap solution in quantity sufficient to neutralize the re-precipitating tendency of said matter, and then adding to the ore while still in contact with the soap solution some agent to precipitate the soap, whereby to leave the treated ore in condition to be subjected to a cyanide treatment.

6. The process of treating carbonaceous gold ore which consists of adding thereto a soluble saponaceous compound to protect the gold from the action of the carbonaceous matter, and permitting the gold to be dissolved and extracted by cyanide.

7. The process of treating gold and silver bearing ores containing carbonaceous matter, consisting of treating the ore in a pulverized condition with a soap solution in combination with an acid, and then subjecting the ore to the action of cyanide.

8. The process of treating gold and silver ores containing some substance causing a

premature precipitation of the precious metals from a cyanide solution, consisting in previously adding thereto a semi-colloidal solution of a fatty acid salt to protect the gold and silver from being prematurely precipitated by said substance, and then removing the precious metals in solution with an alkaline cyanide, and finally treating this effluent solution for the recovery of the precious metals.

9. The process of treating gold and silver

bearing ores containing graphitic or carbonaceous matter, consisting of concentrating the precious metal content by means of flotation, and then treating the flotation concentrates with a soluble saponaceous reagent, after which cyanide is applied to dissolve the precious metals.

In testimony whereof I affix my signature.

FRANK M. DARROW.